

## UNITED STATES PATENT OFFICE

GEORGE RIVAT, OF PATERSON, NEW JERSEY, ASSIGNOR TO CELANESE CORPORATION OF AMERICA, A CORPORATION OF DELAWARE

TREATMENT OF MATERIAL CONTAINING DERIVATIVES OF CELLULOSE AND PRODUCT THEREOF

No Drawing.

Application filed June 21, 1929. Serial No. 372,802.

This invention relates to the treatment of materials containing organic derivatives of cellulose whereby their affinity towards certain dyestuffs is altered.

5 An object of my invention is to treat material and particularly textile material containing organic derivatives of cellulose with certain nitrogen compounds that tend to alter the affinity of such materials towards 10 certain dyestuffs. Other objects of my invention will appear from the following detailed description.

I have found that if materials containing organic derivatives of cellulose and particularly cellulose acetate are treated with certain organic nitrogen compounds, particularly triethanol amine, their affinity towards certain dyestuffs, particularly basic dyestuffs, is altered, such affinity being generally 20 reduced. I employ this discovery for the production of differential color effects as will be more specifically described.

In accordance with my invention I treat materials, particularly textile materials 25 containing yarns of organic derivatives, with certain nitrogen compounds that alter their affinity towards certain dyestuffs, which treatment may be local or over the entire surface. The so treated material may 30 then be treated with the dye whereby many ornamental effects may be obtained.

While this invention is applicable to the treatment of materials containing organic derivatives of cellulose in general, such as 35 organic esters of cellulose or cellulose ethers, it will be described more particularly with respect to the treatment of textile materials containing yarns of cellulose acetate. Examples of other organic esters of cellulose 40 are cellulose formate, cellulose propionate and cellulose butyrate while examples of cellulose ethers are ethyl cellulose, methyl cellulose and benzyl cellulose.

The material to be treated may be in the 45 form of yarn or it may be in the form of fabric. If yarn is to be treated it may be immersed in the form of hanks or wound onto bobbins, cones or other packages in a bath containing the treating agent. If in 50 the form of fabric it may be immersed in

such bath, but preferably the treating agent is applied locally to the fabric by printing or stencilling in order to obtain the resist printing effect upon a subsequent application of the dyestuff.

55 The nitrogen containing agent that alters the affinity of the cellulose acetate material is preferably triethanol amine  $N(CH_2CH_2OH)_3$  or salts thereof formed by neutralizing the same with acids such as sulfuric acid or acetic acid. However, I have found that other nitrogen compounds such as diethanol amine,  $NH(CH_2CH_2OH)_2$ , pyrrol, pyridine or dimethyl aniline are also effective for this purpose, but to a considerably less extent than is triethanol amine. The triethanol amine employed may have diethanol amine or mono ethanol amine admixed therewith.

60 In applying the triethanol amine in the form of a bath, it may be employed as an aqueous solution containing from less than 0.5 to 2.0% or more of the same, the temperature preferably being from 65 to 90° C., and the time of treatment being from 10 65 minutes or less to 25 minutes or more.

70 This invention may be employed to produce resist or reserve printing effects. In this case the triethanol amine or similar agent is incorporated in suitable amounts in a 75 printing paste containing the usual thickeners such as gum tragacanth, gum arabic or British gum, examples of suitable amounts being from less than 10 to 30 or more grams of triethanol amine per liter of printing 80 paste. After the local application of this paste, the fabric is steamed in open steam for 10 to 30 minutes and is then washed. The fabric so treated has a differential affinity 85 for certain dyestuffs and differential color 90 effects may be produced. Thus if the fabric is so treated in a bath containing dyestuffs, the affinity towards which is decreased by treatment with triethanol amine, resist or discharge effects are produced, i. e. lighter 95

color designs on darker background.

If designs of one color on a background of another color are desired, such as ordinarily produced by color discharge printing, there 100 may be incorporated in the printing paste

containing the triethanol amine or similar acting materials a dye for the fabric being treated. After the steaming or ageing and subsequent washing of the fabric so treated 5 it may be dyed with a dyestuff of another color whose affinity towards the treated portion is diminished, thus producing designs of one color against a background of a different color.

- 10 Beautiful cross-dye or differential color effects may be produced by associating together yarns of cellulose acetate that have been treated with the triethanol amine or similar substance with untreated yarns of 15 cellulose acetate in any desired pattern. Thus two kinds of yarns may be woven together by means of jacquard or similar looms to produce any desired pattern, or they may alternate in the warp and/or weft in any 20 desired manner. When the fabric so formed is subjected to a dye bath containing a dyestuff towards which its affinity is altered by treatment with the triethanol amine, differential color effects are produced.
- 25 As to the dyestuff towards which cellulose acetate textile material that has been treated with triethanol amine or similar substances has a diminished affinity, a large number of basic and certain direct and acid dyestuffs have been found to have this property.

30 Examples of basic dyestuffs which have a greatly diminished affinity for cellulose acetate material treated with triethanol amine are:

|                   | Group A | Schultz No. |
|-------------------|---------|-------------|
| 35 Methylene blue | 659     |             |
| Capri blue        | 620     |             |
| Pyronine G        | 568     |             |
| Malachite green   | 495     |             |
| 40 Auramine       | 493     |             |

45 Examples of basic dyestuffs that have a diminished affinity, but whose affinity is not diminished to as great an extent as Group A are:

|                                                                           | Group B | Schultz No. |
|---------------------------------------------------------------------------|---------|-------------|
| 50 Chrysoidine                                                            | 36      |             |
| Phosphine                                                                 | 606     |             |
| Thioflavine                                                               | 618     |             |
| Fuchsin                                                                   | 512     |             |
| Methyl violet                                                             | 518     |             |
| Saframine                                                                 | 679     |             |
| Dianisidine (diazotised and developed with beta hydroxyl naphthoic acid). |         |             |

55 Examples of basic dyestuffs whose affinity to cellulose acetate material which has been treated with thiethanol amine is increased are:

|                   | Group C | Schultz No. |
|-------------------|---------|-------------|
| 60 Methylene grey | 681     |             |
| Acridin orange    | 603     |             |

In order further to illustrate my invention but without being limited thereto, the following specific examples are given.

### Example I

70 Yarn of an acetone soluble cellulose acetate in the form of hanks are immersed in an aqueous solution containing 10 to 15 grams of triethanol amine per liter at a temperature of 70 to 80° C. for 15 minutes. The yarn so treated is woven with untreated yarn of cellulose acetate into a fabric of any desired construction and the fabric thus formed is treated in a dye bath containing any of the dyestuffs of Group A. If the amount of dyestuff present is relatively small the yarn that has been treated with the triethanol amine is substantially undyed while the untreated yarn is dyed thus producing beautiful effects of mixed color and white.

### Example II

75 A fabric consisting wholly of acetone soluble cellulose acetate yarn is printed with a paste containing 10 to 20 grams of triethanol amine per liter and gum tragacanth as thickener. The paste is locally applied by means of printing rollers for desired designs engraved thereon. The fabric after application of the paste is steamed for 15 to 20 minutes in open steam, washed and then dyed with a bath containing any of the dyes of Group A. Substantially white designs on a 80 colored background are produced.

85 It is to be understood that the foregoing detailed description is given merely by way of illustration, and that many variations may be made therein without departing from the 90 spirit of my invention.

Having described my invention, what I claim and desire to secure by Letters Patent is:

1. Method of altering the affinity of materials containing organic derivatives of cellulose towards certain dyestuffs comprising treating at least part of said material containing the organic derivative of cellulose with a substance, selected from the group consisting of ethanolamines and their salts, capable of altering said affinity.

105 2. Method of altering the affinity of materials containing organic esters of cellulose towards certain dyestuffs comprising treating at least part of said material containing the organic ester of cellulose with a substance, selected from the group consisting of ethanolamines and their salts, capable of altering said affinity.

110 3. Method of altering the affinity of materials containing cellulose acetate towards certain dyestuffs comprising treating at least part of said material containing the cellulose acetate with a substance, selected from the group consisting of ethanolamines and their salts, capable of altering said affinity.

115 4. Method of altering the affinity of material containing organic derivatives of cellulose towards certain dyestuffs comprising

70

80

85

90

95

100

105

110

115

120

125

130

treating at least part of said material containing the organic derivative of cellulose with a substance selected from a group consisting of triethanol-amine and its salts.

5. Method of altering the affinity of material containing cellulose acetate towards certain dyestuffs comprising treating at least part of said material containing the cellulose acetate with a substance selected from a group

10 consisting of triethanol amine and its salts.

6. Method of coloring a textile material containing yarns of cellulose acetate comprising treating at least part of the textile material with a substance, selected from the group

15 consisting of triethanol amine and its salts, capable of altering its affinity towards certain dyestuffs and then treating the textile material with such dyestuffs.

7. Method of coloring textile materials

20 containing yarns of cellulose acetate comprising treating at least part of the textile material with a substance, selected from the group consisting of triethanol amine and its salts, capable of decreasing its affinity to

25 wards certain basic dyestuffs and then treating the textile material with such basic dye-  
stuffs.

8. Method of producing differential color effects comprising locally applying to fabric

30 containing yarns of organic derivatives of cellulose, a material, selected from the group consisting of triethanol amine and its salts, which is capable of altering its affinity towards certain dyestuffs and then dyeing the

35 treated material with such dyestuffs.

9. Method of producing differential color effects comprising locally applying to fabric containing yarns of cellulose acetate, a material, selected from the group consisting of

40 triethanol amine and its salts, which is capable of altering its affinity towards certain dye-  
stuffs and then dyeing the treated material with such dyestuffs.

10. Method of producing differential color

45 effects comprising locally applying to a fabric containing yarns of cellulose acetate, a material, selected from the group consisting of triethanol amine and its salts, which is capable of decreasing its affinity towards cer-

50 tain basic dyestuffs and then dyeing the treated material with such dyestuffs, whereby the treated parts are lighter in color.

11. Materials containing derivatives of cel-  
lulose at least part of which has been treated

55 with a substance selected from the group con-

sisting of ethanolamines and their salts, ca-

pable of altering its affinity towards certain

dyestuffs.

12. Materials containing cellulose acetate

60 at least part of which has been treated with a substance, selected from the group consist-

ing of ethanolamines and their salts, capable

of altering its affinity towards certain dye-  
stuffs.

65 13. Material containing yarns of cellulose

acetate at least part of which has been treat-  
ed with a substance, selected from the group

70 consisting of triethanol amine and its salts,

capable of altering its affinity towards cer-

tain dyestuffs.

In testimony whereof, I have hereunto sub-

scribed my name.

GEORGE RIVAT.

75

80

85

90

95

100

105

110

115

120

125

130